

J. C. McCLINTOCK & R. J. SHOEMAKER.  
PROCESS FOR LEAD PLATING METALS.  
APPLICATION FILED JUNE 26, 1915.

1,195,376.

Patented Aug. 22, 1916.



WITNESSES

*Edw. Thorper*  
*B. J. Hoff*

INVENTORS  
*J. C. McClintock*  
*R. J. Shoemaker*  
BY *Myndea*  
ATTORNEYS

# UNITED STATES PATENT OFFICE.

JOHN CALHOUN McCINTOCK AND ROBERT JAY SHOEMAKER, OF TOPEKA, KANSAS.

## PROCESS FOR LEAD-PLATING METALS.

1,195,376.

Specification of Letters Patent. Patented Aug. 22, 1916.

Application filed June 26, 1915. Serial No. 36,466.

*To all whom it may concern:*

Be it known that we, JOHN C. McCINTOCK and ROBERT J. SHOEMAKER, citizens of the United States, and residents of Topeka, in the county of Shawnee and State of Kansas, have invented a new and Improved Process for Lead-Plating Metals, of which the following is a full, clear, and exact description.

- 10 Our invention relates to a process for lead-plating metals and consists in depositing lead in an adherent, uniform and non-porous coating on metals, more particularly iron and steel.
- 15 The process is based on the fact that metals, after a suitable cleansing of impurities on their surfaces, if dipped into molten lead at a proper temperature will become coated with lead, which adheres to the surface of the metal and forms a non-porous and uniform coating. The process of lead plating is greatly improved if the metal is dipped into a molten flux of zinc chlorid previous to its immersion into the lead bath.
- 20 25 The details of our process will be described in connection with iron or steel; but it is self-evident that any other metal, the melting point of which is above the temperature of the lead bath, can be coated similarly.
- 30 35 The iron or steel to be coated with lead is cleaned from inorganic impurities, and particularly of oxids of iron, by immersing the iron or steel in a bath consisting preferably of equal parts by weight of commercial hydrochloric acid and water. This acid bath is maintained at a temperature of approximately 70° F. Care must be exercised that the metal receives a thorough cleaning in the bath in order to remove all oxids, as any 40 45 oxid remaining on the surface of the iron will make the lead coating porous and, therefore, the metal will not be properly protected by the coating formed.

In case the surface of the iron or steel contains, in addition to the mineral impurities, organic impurities, like oil, grease, paint, etc., the metal must be immersed in a caustic alkaline solution before it is placed into the acid bath. The caustic solution is preferably 50 55 caustic soda or potash dissolved in ten parts by weight of water and used at a temperature of approximately 212° F. The iron from the acid bath, while covered with the diluted acid, is plunged into the flux of molten zinc chlorid and then into the molten

lead. The temperature of the two baths, that is, of the flux and of the lead, should be between 640 and 680 degrees F. in order to secure satisfactory results.

We have found by experiment that a lead deposit obtained at any other temperature than 640 to 680 degrees F. is not satisfactory. Below 640° the metal does not possess sufficient fluidity to cover the metal uniformly; and above 680° F. the lead oxidizes so rapidly that it is impossible to secure a deposit free from burned spots, "pin holes," or other serious defects which expose the surface of the metal coated.

The appended drawing shows diagrammatically a preferred form of a furnace to be used in connection with our process. The chamber A is heated, preferably by a gaseous fluid fuel to easily regulate the temperature of the molten lead within. Extending 70 slightly below the surface of the lead within the chamber A, and also above the level of the lead, is a frame B of any suitable form and preferably secured to one side of the chamber in the furnace. Said frame forms 75 a compartment for the flux or molten zinc chlorid. The flux, by reason of its density, will flow upon the surface of the lead, and its level above the lead surface is controlled 80 by the walls of the frame B. The surface of the lead is kept clean by skimming it with any suitable means. In using this furnace, the metal to be coated, after it is cleaned in an acid bath and while the acid covers the 85 surface of the cleaned metal, is plunged into the compartment B and is held in the zinc chlorid until the temperature of the metal to be coated has reached that of the flux, which is between 640 and 680 degrees 90 Fahrenheit.

When the metal has attained the temperature of the flux, it is plunged perpendicularly into the molten lead which lies immediately under the zinc chlorid, that is, the object is forced through the opening in the bottom of the frame B. After the object enters the chamber A, the same is positioned laterally or diagonally under the partition which separates the compartment B from the chamber A, and the object is then extracted from the chamber A.

It is to be noted that the operation of plunging the material for treatment with zinc chlorid perpendicularly into the molten lead removes all adhering zinc chlorid which 110

flows up through the lead and collects in compartment B. In this manner the greater quantity of the zinc chlorid is retained in compartment B and, therefore, will not 5 contaminate the lead in compartment A. This permits the utilization of the zinc chlorid over and over again, and, at the same time, the metal in compartment A is not contaminated with flux.

10 We have found that an alloy of 96% of lead, 2% of antimony, and 2% of tin when deposited upon iron or steel produces a coating of greater hardness, tensile strength, and more crystalline than lead alone, and by the 15 term "lead" as used in the claims we intend to include ordinary lead alloys, such, as for example as that just specified. It is also to be remarked that the melting point of this alloy is lower than that of lead.

20 It is self-evident that the entire process can be carried out by mechanical means in a manner similar to the galvanizing and tinning processes.

25 Our process can be efficiently applied to the coating of sheet metal, pipe, boiler flues, raw wire, worked wire, etc.

While we have described the principle of 30 operation, together with the process which we now consider to be the best embodiment thereof, we desire to have it understood that the process shown is merely illustrative and that such changes may be made as are within the scope of the appended claims.

We claim:

1. A lead-plating process for metals, 35 consisting in cleaning the surface of the metal with an acid, immersing the metal so cleaned, and while it is covered with the acid film, into a molten flux, maintaining the metal immersed until the temperature there- 40 of rises to that of the molten flux, then dipping the metal into a bath of molten lead, which bath is at a temperature substantially that of the flux.

2. A lead-plating process for metals, 45 consisting in submerging the metals in hydrochloric acid to remove all oxids therefrom, then immersing the metal, while it is covered by a film of acid, into molten flux of zinc chlorid supported by a molten lead bath, 50 the temperature of the bath being maintained between 640 and 680° Fahrenheit, maintaining the metal in the flux until its temperature is that of the flux, then lowering the metal into the lead below the flux 55 and extracting the metal from the bath where its surface is clear of the flux.

In testimony whereof we have signed our names to this specification in the presence of two subscribing witnesses.

JOHN CALHOUN McCLINTOCK.  
ROBERT JAY SHOEMAKER.

Witnesses:

W. D. BOUGHTON,  
FRANCES SHOEMAKER.